

# United States Patent Office

3,069,346

Patented Dec. 18, 1962

1

3,069,346

## WAX COMPOSITION

John D. Tench, Prospect Park, Pa., assignor to Sun Oil Company, Philadelphia, Pa., a corporation of New Jersey

No Drawing. Filed Jan. 20, 1959, Ser. No. 787,827

3 Claims. (Cl. 208—21)

This invention relates to a novel paraffin wax composition derived from petroleum and suitable for coating certain fibrous dairy product containers. More particularly, the invention relates to a novel hydrocarbon wax composition composed of three specific paraffin wax components, the composition being particularly suitable for coating fibrous containers used in packaging cottage cheese.

Paraffin waxes have heretofore been prepared and employed for a variety of uses, including the coating of fibrous containers for dairy products. However, such paraffin wax compositions as have heretofore been disclosed have been unsuitable for certain specific dairy applications such as coating containers designed to package cottage cheese. It appears that one or more of the ingredients of cottage cheese in some manner affects the protective wax coating so that thereafter various fluids of the cheese composition are free to pass through the wax barrier. These fluids are then adsorbed by the walls of the fibrous containers, causing the container to become soggy. Cottage cheese containers which have been so-spoiled are subject to considerable consumer resistance. Furthermore, in some instances actual leaks develop in the damaged containers.

Heretofore, in providing wax compositions for coating fibrous cottage cheese containers it has been found necessary to employ various other materials in addition to the paraffin wax to overcome the above-described difficulties. For example, materials such as microcrystalline wax, resin, and the like, have, of necessity, been compounded with paraffin waxes in preparing coating compositions suitable for cottage cheese containers.

The provision of a suitable wax composition for coating fibrous cottage cheese containers is further complicated by the requirement applicable to all wax-coated containers that, when stacked in a nesting relationship, they must not stick together at temperatures normally encountered during storage and shipment. In other words, the "blocking temperature" of the wax composition employed for coating must be relatively high.

A further requirement, applicable to wax-coated containers which are used in packaging consumer goods such as cottage cheese, is that the coated container must present a pleasing appearance to the customer, and retain such appearance for a reasonable length of time. Thus, it is necessary that the wax coating have a high gloss and extended gloss retention, and that the coating be smooth and uniform as well as unbroken.

In view of the above, one object of the present invention is to provide a novel wax composition, and process for preparing it, which composition is composed entirely of petroleum paraffin wax, and which is particularly suitable for coating fibrous cottage cheese containers. Another object is to provide a novel paraffin wax composition which, when applied as a coating to fibrous cottage cheese containers, does not cause such containers to stick together when stored in contact with each other at temperatures of up to 100° F. and higher. A further object is to furnish a novel paraffin wax composition which will provide a smooth, uniform protective coating of high gloss and good gloss retention when applied to fibrous containers designed for packaging cottage cheese. Still another object is to provide fibrous cottage cheese containers coated with the above wax composition.

2

These and other objects and benefits will become more readily apparent from a reading of the following detailed description of the invention.

It has now been discovered that by blending three separate paraffin wax components, all of which are derived from petroleum and have specific properties within narrow ranges, the resulting composition is suitable for coating fibrous containers used for packaging cottage cheese. It is also essential to the practice of the invention that the three paraffin wax components each be employed in specified narrow ranges of concentration, as will appear hereinafter.

As used herein, melting points for paraffin waxes are as determined by ASTM method designated D87-57, penetrations are as determined by ASTM method designated D1321-57T and viscosities (SUS—Saybolt Universal seconds) are as determined by ASTM method designated D446-53, unless otherwise stated.

The first paraffin wax component used in the present compositions must have a melting point of from 130° F. to 136° F., a penetration at 100° F. of from 30 to 50 and viscosity at 210° F. of from 36 to 39 SUS. On vacuum distillation, 5 percent of the wax should be distilled at a temperature equivalent to about 750° F. at atmospheric pressure, and 95 percent should be distilled at a temperature equivalent to about 820° F. at atmospheric pressure. This wax is prepared from petroleum by distilling slack wax from the dewaxing of lubricating oil, or a topped, high wax-content crude petroleum, and collecting the fraction distilling between about 390° F. and 475° F. at 2 mm. of mercury absolute pressure. This distillate fraction is dissolved in a solvent such as an equimolar mixture of methyl ethyl ketone and benzene at an elevated temperature. Preferably, about four parts by volume of solvent per part of the wax fraction is employed. The resulting solution is then cooled to from about 32° F. to about 37° F., and the wax which precipitates at this temperature is separated from the liquid by means such as filtration. Advantageous, the wax is washed, at the temperature of precipitation, with an additional quantity of the same solvent. Upon removal of the wash solvent, the recovered paraffin wax forms the first paraffin wax component of the present composition.

The second paraffin wax component must have a melting point of from 125° F. to 132° F., a penetration at 100° F. of from 80 to 120, and a viscosity at 210° F. of from 38 to 40. This particular paraffin wax is not suitable for sole use in coating fibrous containers unless kept under refrigeration because it readily blocks, both in the form of wax slabs and when formed as a coating on the containers, the blocking temperature being about 90° F. or lower. The paraffin wax component meeting the above specifications can be prepared by two methods. In the first method of preparation, a slack wax such as is obtained from the dewaxing of lubricating oil, and which may still contain approximately 30 percent oil, is vacuum distilled, and the fraction distilling between about 390° F. to about 565° F. at 2 mm. of mercury absolute pressure is collected. This fraction is dissolved in a solvent which is preferably a mixture of methyl ethyl ketone and benzene in about equal volumes, solution being effected at a temperature of from about 165° F. to about 195° F., and with about 6 parts by volume of the solvent per part of the wax fraction being used. The solution is slowly cooled to a temperature of from about 75° F. to about 83° F., and the wax which precipitates at this temperature is separated by means such as filtration. The solution separated from the precipitated wax is further slowly cooled to a temperature of from about 25° F. to about 33° F., and the wax which precipitates at this lower temperature, after separation by means such as fil-

tration, forms the second paraffin wax component of the present composition. Advantageously, the wax after separation from the solution is washed, preferably with additional solvent and at about the same temperature as filtration, e.g., from 28° F. to 32° F., and the wax is then again separated and recovered.

An alternate method for preparing the second paraffin wax component of the present invention provides considerable flexibility in obtaining a wax product of the desired properties. This method comprises separating from slack wax two distillate fractions, one of which distills in the range of from about 390° F. to about 475° F. at 2 mm. of mercury absolute pressure, and a second fraction distilling in the range of from about 450° F. to about 565° F. at 2 mm. of mercury absolute pressure. As usually occurs, the initial boiling point of the second fraction will overlap, to some extent, the end boiling point of the first-mentioned distillate fraction. The lower boiling distillate fraction is dissolved in a suitable solvent at an elevated temperature, as above described, with about 6 parts by volume of the solvent per part of the wax fraction being used, and the solution is slowly cooled to a temperature of from about 25° F. to about 32° F. The wax which precipitates at this temperature is then separated by means such as filtration. The higher boiling distillate fraction is also dissolved in a suitable solvent at an elevated temperature, as above described, about 4.5 parts by volume of solvent per part of the wax fraction being used, and the solution is slowly cooled to a temperature of from about 72° F. to about 82° F. The wax which precipitates at this temperature is separated by means such as filtration, and is not further used in the practice of this invention. The remaining solution is further slowly cooled to a temperature of from about 25° F. to about 33° F. The wax precipitated at this latter temperature is then separated by means such as filtration. The two distillate waxes prepared as above described are combined to form the second paraffin wax component of the present invention. Considerable flexibility is obtained since the blending may be in various proportions so that the properties of the resulting combination are within the limits set forth above for the second paraffin wax component. If desired, the two distillate wax fractions can be washed independently, preferably with an additional quantity of the solvent and at the temperature of the final precipitation, and separated from the solvent prior to blending; or, the wet distillate fractions may be first combined, washed jointly, and then separated. In general, from about 69 to about 75 percent of the second paraffin wax component will consist of wax from the lower boiling distillate fraction since, as has been found, such proportions give a wax having properties within those specified as essential for the second paraffin wax component of the invention.

The third paraffin wax component employed in the practice of this invention must have a melting point of from 149° F. to 155° F., a penetration at 130° F. of from 35 to 65 and a viscosity at 210° F. of from 42 to 46 SUS. On vacuum distillation, 5 percent of this wax should be distilled at a temperature equivalent to about 850° F. at atmospheric pressure, and 95 percent should be distilled at a temperature equivalent to about 950° F. at atmospheric pressure. This wax is prepared from petroleum by distilling a slack wax, which may be from the dewaxing of lubricating oil or from a topped, high wax-content crude petroleum, and collecting the fraction distilled between about 450° F. and 565° F. at 2 mm. of mercury absolute pressure. This distillate fraction is dissolved in a solvent such as an equimolar mixture of methyl ethyl ketone and benzene at an elevated temperature. Preferably, about two parts by volume of solvent per part of wax fraction is employed. The resulting solution is then cooled to a temperature of from about 77° F. to about 83° F., and the wax which precipitates at this temperature is separated by means such as filtra-

tion. Advantageously, the wax is washed, preferably with an additional quantity of the solvent and at the temperature of precipitation, and then separated from the solvent. The recovered wax forms the third paraffin wax component of the invention.

As above stated, it is essential that the above-described paraffin wax components of the novel composition of this invention be present in specific amounts. The first paraffin wax component must constitute from 50 to 60 percent by weight; the second paraffin wax component must constitute from 25 to 35 percent by weight; and the third paraffin wax component must constitute from 12 to 18 percent by weight, all percentages being based on the final composition. If the quantity of either of the relatively low-melting paraffin wax components (viz., the first and second components) is below the stated range, poor coverage of the paper containers results and leakage of the container may occur. Furthermore, if a quantity of such waxes above the stated range is used, blocking of the coated articles is experienced even at relatively low temperatures. If the quantity of the relatively high-melting paraffin wax component (viz., the third component) is below the stated minimum concentration, the coated containers will also exhibit poor blocking characteristics. If the quantity of the latter component is above the stated maximum concentration, the coated articles will present an unsightly appearance in that the surface exhibits serpentine lines and poor gloss.

In addition to requiring critical amounts of each component, as above described, it appears that waxes having properties outside of the stated ranges for each paraffin wax component cannot be used. For example, substitution of a wax having a melting point lower than the range designated for either of the lower-melting paraffin wax components completely defeats the purposes of the invention in that the resulting composition exhibits poor blocking characteristics, and hence is unsuitable for coating fibrous articles. Likewise, substitution of a higher-melting paraffin wax having properties outside of the ranges described above for the higher-melting paraffin wax component of the present invention results in a composition exhibiting one or more of the above-described difficulties. The final composition of the invention will have a melting point of from about 132° F. to about 137° F., a penetration at 100° F. of from about 40 to about 60, and a viscosity at 210° F. of from about 38.0 to about 39.5 SUS.

In order to demonstrate a specific embodiment of the present invention, and the advantages thereof, three paraffin waxes were prepared as follows:

The first paraffin wax component has a melting point of 134° F., a penetration at 100° F. of about 40 and a viscosity at 210° F. of 38.1 SUS and is prepared as described below. On vacuum distillation, 5 percent of this wax is distilled at a temperature equivalent to about 750° F. at atmospheric pressure, and 95 percent is distilled at a temperature equivalent to about 820° F. at atmospheric pressure. Specifically, this wax is prepared by topping a high wax-content crude petroleum to about 38 percent bottoms. The bottoms are charged to a vacuum distillation operation which operates at 2 mm. of mercury absolute pressure, and the fraction distilling between 390° F. and 475° F. is collected. This distillate fraction is dissolved in a solvent consisting of a mixture of about 60 volume percent methyl ethyl ketone and 40 volume percent benzene at a temperature of about 180° F., about 4 parts by volume of the solvent per part of wax being used. The resulting solution is slowly cooled to a temperature of about 35° F., and the wax precipitated at this temperature is separated by filtration. The wax cake is further washed with an additional quantity of the above solvent at a temperature of 35° F., and the wax is then recovered from the solvent.

The second paraffin wax component is prepared from

slack wax obtained by dewaxing lubricating oil. The slack wax contains about 30 percent residual oil. This slack wax is distilled at a pressure of 2 mm. mercury absolute and two distillate fraction are collected, one boiling in the range of from about 390° F. to about 475° F., and the other boiling in the range of from about 450° F. to 565° F., at 2 mm. of mercury absolute pressure. The lower boiling fraction is dissolved in an equimolar mixture of methyl ethyl ketone and benzene at a temperature of about 170° F., 6 parts by volume of solvent being used per part of the wax fraction. The resulting solution is slowly cooled to a temperature of 28° F., and the precipitated wax is recovered by filtration. After washing with additional solvent at 28° F., the wax is again recovered by filtration. The higher boiling distillate fraction is dissolved in a similar solvent, with 4.5 parts by volume of the solvent per part of the wax fraction being used, and the resulting solution is cooled to 80° F. The precipitated wax is separated by filtration and discarded, and the filtrate is further cooled to 30° F. The wax separating at this latter temperature is separated by filtration, washed with an additional quantity of solvent at 30° F., and then separated from the solvent by filtration. The two so-formed waxes are blended in quantities such that the final composition contained 72 percent of wax derived from the lower-boiling distillate fraction and 28 percent derived from the higher boiling distillate fraction. This blend constitutes the second paraffin wax component of the invention. This component has a melting point of 127° F., a viscosity at 210° F. of 39.0 SUS and a penetration of 100° F. of about 100.

The third paraffin wax component of the invention, having a melting point of 151° F., a viscosity at 210° F. of 43.6 SUS and a penetration at 130° F. of about 50 is prepared as described below. On vacuum distillation, 5 percent of this wax distills below a temperature equivalent to 820° F. at atmospheric pressure, and 95 percent distills below a temperature equivalent to 950° F. at atmospheric pressure. Specifically, this wax is prepared by topping a high wax-content crude petroleum to about 38 percent bottoms. The bottoms are charged to a vacuum distillation operation, which operates at 2 mm. of mercury absolute pressure, and the fraction distilling between about 450° F. and about 565° F. is collected. This distillate fraction is dissolved in a solvent consisting of a mixture of 60 volume percent methyl ethyl ketone and 40 volume percent benzene at a temperature of about 180° F., about 2 parts by volume of solvent per part of wax being used. The resulting solution is slowly cooled to a temperature of 80° F., and the wax precipitated at this temperature is separated by filtration. The wax cake is then washed with an additional quantity of the same solvent at a temperature of 80° F., and the wax is recovered from the solvent by filtration. The recovered wax constitutes the third paraffin wax component of the invention.

The three paraffin wax components are blended together by heating a mixture thereof to a temperature of about 200° F., with stirring. The quantities of the individual components employed are such that the resulting composition contains 55 percent of the first paraffin wax component, 30 percent of the second paraffin wax component and 15 percent of the third paraffin wax component, all percentages being expressed on a weight basis. The final composition has a melting point of 134° F., a penetration at 100° F. of about 50 and a viscosity at 210° F. of 38.5 SUS. The above-prepared wax composition is employed in coating fibrous cottage cheese containers. Application to the containers is made in conventional equipment without unusual difficulties. Good coverage is obtained in all cases, and the resulting coated containers present a pleasing appearance, exhibiting high gloss and good gloss retention, and they do not block even at temperatures of up to 100° F. Furthermore, when cottage

cheese containers are coated with the wax composition of this invention, no evidence of deterioration of the coating or of consequent leakage due to contact with cottage cheese is experienced even after long periods of storage.

In preparing the three components of the paraffin wax composition of this invention, the operating conditions specified herein must be carefully observed in order to secure the advantages of the invention. However, in one respect, some variation may be practiced and good results still obtained. Specifically, the solvent employed for dissolution of the wax fractions can be varied both as to the nature of its components and their respective proportions. Thus the solvent described, consisting of approximately equal parts by volume of methyl ethyl ketone and benzene, gives good results, but more or less of these two constituents, e.g. from about 30 to about 70 percent by volume of benzene, can also be used. Furthermore, other solvents can replace either methyl ethyl ketone or benzene, for example toluene can be substituted for a portion of the benzene and good results obtained.

This invention is to be distinguished from that disclosed in my copending patent application Serial Number 787,822 of even filing date wherein I have disclosed a paraffin wax composition, consisting of the same three wax components but in substantially different proportions, especially suitable for use as the wax ingredient of candle compositions. In that application, I disclose a composition consisting of from 32 percent to 42 percent by weight of the component herein termed the first paraffin wax component; from 45 percent to 55 percent by weight of the component herein termed the second paraffin wax component; and from 10 percent to 16 percent by weight of the component herein termed the third paraffin wax component. The latter composition is not suitable for use in coating fibrous cottage cheese containers in accordance with the instant invention, nor is the composition herein disclosed suitable for use in candle compositions as contemplated by my copending application.

The invention claimed is:

1. A wax composition consisting essentially of: (A) from 50 percent to 60 percent by weight of a paraffin wax derived from petroleum slack wax and having a melting point of from 130° F. to 136° F., a penetration at 100° F. of from about 30 to about 50 and a viscosity at 210° F. of from 36 to 39 SUS; (B) from 25 percent to 35 percent by weight of a paraffin wax derived from petroleum slack wax and having a melting point of from 125° F. to 132° F., a penetration at 100° F. of from about 80 to about 120 and a viscosity at 210° F. of from 38 to 40 SUS; and (C) from 12 percent to 18 percent by weight of a paraffin wax derived from petroleum slack wax and having a melting point of from 149° F. to 155° F., a penetration at 130° F. of from about 35 to about 65 and a viscosity at 210° F. of from 42 to 46 SUS.

2. A wax composition according to claim 1 wherein the paraffin wax of (A) constitutes about 55 percent by weight; the paraffin wax of (B) constitutes about 30 percent by weight; and the paraffin wax of (C) constitutes about 15 percent by weight.

3. Process for preparing a wax composition suitable for coating fibrous cottage cheese containers which comprises: (A) distilling slack wax and separating the fraction distilling in the range of from about 390° F. to 475° F. at 2 mm. of mercury absolute pressure, dissolving the separated wax fraction in a solvent at an elevated temperature, cooling the resulting solution to a temperature of from about 32° F. to 37° F., and separating the precipitated wax as a first paraffin wax component having a melting point of from 130° F. to 136° F. and a penetration at 100° F. of from about 30 to about 50; (B) distilling slack wax and separating a fraction distilling in the range of from about 390° F. to 475° F. at 2 mm. of mercury absolute pressure and a fraction distilling in the

range of from about 450° F. to 565° F. at 2 mm. of mercury absolute pressure, dissolving the lower-boiling fraction in a solvent at an elevated temperature, cooling the resulting solution to a temperature of from about 25° F. to about 32° F. and separating the precipitated wax; 5 dissolving the higher-boiling fraction in a solvent at an elevated temperature, cooling the solution to a temperature of from about 72° F. to 82° F. and separating the precipitated wax, further cooling the solution to a temperature of from about 25° F. to 33° F. and separating the precipitated wax, combining the first-mentioned separated wax with the last-mentioned separated wax to form a second paraffin wax component having a melting point of from 125° F. to 132° F. and a penetration at 100° F. of from about 80 to about 120; (C) distilling slack 15 wax and separating a fraction distilling in the range of from about 450° F. to 565° F. at 2 mm. of mercury absolute pressure, dissolving the separated wax fraction in a solvent at an elevated temperature, cooling the resulting solution to a temperature of from about 77° F. 20 to 83° F. and separating the precipitated wax as a third

paraffin wax component having a melting point of from 149° F. to 155° F. and a penetration at 130° F. of from about 35 to about 65; (D) blending in the molten state the paraffin wax components obtained in steps (A), (B) and (C) in quantities so that the final composition contains, in percent by weight, from 50 percent to 60 percent of said first paraffin wax component, from 25 percent to 35 percent of said second paraffin wax component and from 12 percent to 18 percent of said third paraffin wax component.

## References Cited in the file of this patent

## UNITED STATES PATENTS

|           |               |       |                |
|-----------|---------------|-------|----------------|
| 2,670,323 | Hunter        | ----- | Feb. 23, 1954  |
| 2,756,180 | Perry et al.  | ----- | July 24, 1956  |
| 2,761,814 | Post          | ----- | Sept. 4, 1956  |
| 2,773,812 | Tench         | ----- | Dec. 11, 1956  |
| 2,906,443 | Harvey et al. | ----- | Sept. 29, 1959 |
| 2,915,451 | Bartay        | ----- | Dec. 1, 1959   |